

June 24, 1930.

L. KIRSCHBRAUN

1,765,839

COMPOSITION BOARD

Filed Jan. 24, 1927



Fig. 1



Fig. 2



Fig. 3



Fig. 4 Inventor:

Lester Kirschbraun.

by  
Lester Kirschbraun  
Attest.

Fig. 5



## UNITED STATES PATENT OFFICE

LESTER KIRSCHBRAUN, OF LEONIA, NEW JERSEY, ASSIGNOR, BY MESNE ASSIGNMENTS,  
TO THE PATENT AND LICENSING CORPORATION, OF BOSTON, MASSACHUSETTS, A  
CORPORATION OF MASSACHUSETTS

## COMPOSITION BOARD

Application filed January 24, 1927. Serial No. 163,000.

The object of this invention is to provide a composition board of sufficient durability and strength for use in various capacities, such for example in packaging fabricated roofing elements such as strip shingles which are ordinarily made of roofing felt impregnated and coated with asphalt and covered with granulated mineral. Heretofore it has been customary in packaging 5 such roofing elements for shipment to assemble a suitable number of them, place a thin wooden board on each side of the bundle, and then to secure the package by two or more loops of wire or equivalent 10 binding strand passed around the package and secured in closed loops. While wooden boards are in many ways desirable for this purpose, they are at the same time objectionable on account of their tendency to 15 curl, warp and split, resulting in a material loss. Furthermore, wood is becoming more difficult to obtain and is steadily increasing in price. By my invention, I provide a product which may be utilized as a substitute 20 for the wooden packaging boards, which is in many ways superior to the wood, and is also obtainable in practically unlimited quantities at a comparatively low 25 figure.

30 My invention consists briefly in treating sheets of relatively high bibulous character, as for example roofing felt, in such manner as to substantially thoroughly impregnate the sheets with a saturating material which 35 will dry to a rigid gel-like structure surrounding the fibers of the sheet. As an example of a material of this character which is readily obtainable, I may name sodium silicate. Two or more such sheets 40 after being impregnated with material of the character indicated, are preferably stuck together with an adhesive, which may also by preference be sodium silicate,—this operation 45 being assisted by means of suitable pressure and elevated temperature. The resulting laminated sheet is stiff and durable, having comparatively great strength and high water-resistant properties. This 50 structure is admirably suited for use in

various capacities where thin wooden board is now utilized.

As a specific example, the product of the present invention may be employed as a packaging board for roofing elements. 55 Inasmuch as the composition board embodying my invention is preferably constituted of roofing felt, it can be readily produced in the very industry in which it finds a 60 desirable use.

Further features of my improved composition board will appear from the following description and from the drawing, of which:—

Figure 1 shows one use to which the product of the present invention may be put, and is a perspective of a package of strip shingles with one corner of the shingles broken away to indicate more clearly the 65 protective packaging boards on the side 70 faces of the bundle.

Figure 2 is a fragmentary section of one form of my improved composition board.

Figure 3 is a fragmentary section of another form of board embodying my invention. 75

Figure 4 shows a packaging board having metal ware pieces attached to the edges thereof.

Figure 5 shows in perspective one form 80 of wear piece.

Referring to the drawings in detail, the board 11 is preferably composed of one or more layers of bibulous sheets which can be saturated to a high degree, as for example 85 roofing felt such as is customarily used in the fabricated roofing industry as a foundation or base for asphalt-impregnated roofing elements. For certain uses, one layer of material may be found sufficient, 90 while for others, two or more such layers securely stuck together will be found desirable. In Figure 2 a board comprising two layers is illustrated, each layer consisting of a sheet 13 of roofing felt or similar material having a highly porous or bibulous character, substantially completely impregnated with sodium silicate or other material which on drying will form a gel-like 95 structure surrounding the fibers of the sheet. 100

The dried sheets of felt are then stuck together with suitable adhesive, preferably sodium silicate. A film 14 of the adhesive is indicated in Figure 2, the thickness of the felt being considerably exaggerated. It is preferable to stick the laminae together with a very thin film of silicate, assisting the union of the sheets by subjecting the plied board to pressure and elevated temperature. 5 While only two sheets of felt are illustrated in Figure 2, it is obvious that three or more may be combined in the same way to build up a laminated sheet of any desired thickness according to the strength required. The 10 resultant structure is characterized by its relatively great rigidity and toughness. 15

Although thoroughly dried sodium silicate is somewhat water-resistant, it may be desirable to supply a board which is still further protected against deterioration by moisture. To this end, I may provide facing layers of any desired waterproof or water-resistant material, preferably sticking such layers to the felt laminae with sodium silicate or asphalt as an adhesive. For 20 such facing layers, I find waterproofed paper satisfactory. Such paper for example may consist of a number of plies, one or more of which have been treated with emulsified asphalt in the stock chest of the paper machine or may consist of a plied paper having an interposed film of coalesced bitumin. Asphalt emulsion, such as that known as K-B, are miscible with 25 the wet pulp in a paper machine and can be deposited with the pulp on the paper-forming wire screen. When the paper is dried, the microscopic globules of asphalt which have been held in suspension coalesce, and 30 thus render the ply of the paper which contains them highly water-resistant. Figure 3 illustrates a composition board made by sticking together two sheets of roofing felt which have previously been saturated with sodium silicate and dried. To one or both 35 faces of the laminated board is applied a facing layer of paper 15 having a water-resistant ply 16 which as shown in Figure 3 is preferably deposited next to the ply of the board to which the paper is stuck. It 40 is obvious that the number and arrangement of plies in the water-resistant paper can be varied, also that such paper facing layers may be applied to laminated boards 45 built up of any desired number of laminae. If more complete protection of the laminae against moisture is desired, the water-repellent paper facing layer may be extended over the edges of the boards after the latter 50 have been cut to shape.

A bundle of roofing elements such as strip shingles are indicated at 10, this bundle of shingles having protective packaging boards 11 made of saturated roofing felt as hereinafter described. The package

is held together as by suitable wires or strands 12 which are passed around the package and secured in closed loops.

In order to protect the side edges of the composition board from being cut into by the binding strands 12, I may secure thereto suitable wear pieces 17, preferably of metal as shown in Figure 5, to serve as contact areas for the binding wires at the edges of the board. If flat strips of metal or other material are used for binding the bundles, such wear pieces may not be considered necessary.

My improved composition board is simple and easy to make, can be produced at a very low cost from materials readily obtainable in practically unlimited quantities, is tough and durable in use, and is admirably adapted for the special purpose herein indicated, namely, the packaging of bundles of roofing elements, as well as wall board, panel board, and as a base for a rigid roofing element. In this latter case, it may be coated with asphaltic material and thereafter surfaced with a suitable comminuted material.

An invention may be carried out in which the bibulous roofing felt is saturated at an elevated temperature with molten sulphur and plied together, the excess sulphur on the surface of the felt acting as a cementing medium. The outer plies may be finished with untreated thin paper which, as in the treatment described above, is adapted for printing.

Having thus described certain embodiments of my invention, it should be evident to those skilled in the art that various changes and modifications may be made therein without departing from its spirit or scope as defined by the appended claims.

I claim:—

1. A laminated composition board comprising a layer of fibrous roofing felt material having its fibers surrounded by a mineral gel, and a facing layer of paper containing water-resistant material, said layers being stuck together with an adhesive.

2. A laminated composition board comprising a plurality of layers of roofing felt saturated with sodium silicate, said layers being adhesively united in face to face relationship and a facing layer of water resistant paper stuck to a face of said board.

3. A laminated packaging board for fabricated strip shingles comprising a plurality of layers of roofing felt of suitable size and shape impregnated and stuck together with sodium silicate and facing layers of water resistant paper adhesively stuck to the faces of said board.

In testimony whereof I have affixed my signature.

LESTER KIRSCHBRAUN.